

G. MICHAUD & E. DELASSON,  
PROCESS OF MAKING FILAMENTS FOR LIGHTING AND HEATING.  
APPLICATION FILED AUG. 18, 1905.

904,139.

Patented Nov. 17, 1908.



RECEIVED  
L. Goldman  
C. Heymann.

INVENTORS  
Georges Michaud  
Eugène Delasson  
by J. Hinger  
Attorney

# UNITED STATES PATENT OFFICE.

GEORGES MICHAUD AND EUGÈNE DELASSON, OF PARIS, FRANCE.

## PROCESS OF MAKING FILAMENTS FOR LIGHTING AND HEATING.

No. 904,139.

Specification of Letters Patent.

Patented Nov. 17, 1908.

Application filed August 18, 1905. Serial No. 274,717.

To all whom it may concern:

Be it known that we, GEORGES MICHAUD and EUGÈNE DELASSON, both citizens of the Republic of France, and residents of 6 Rue St. Laurent, Paris, France, have invented a Process of Making a Filament for Lighting and Heating, of which the following is a specification.

This invention has for its object to provide an improved process of making a durable and refractory filament obtained by the fusion of magnesia, silica, or alumina.

The process consists generally in feeding suitable finely divided material and particularly powdered alumina and oxids of thorium, cerium and chromium in a fine stream and arresting its movements in a zone of intense heat to agglomerate the same to produce a filament therefrom.

20 The process in its more specific details will be clearly set forth in the description of the operation of apparatus preferably employed in making the filament.

This filament is obtained by means of the apparatus hereinafter described or other equivalent arrangement, in which the necessary conditions of fusion and of feed are fulfilled.

An apparatus which we have found to be particularly well adapted for carrying out our process is illustrated in the accompanying drawings, in which,

Figure 1, is an elevation partly in section and Fig. 2, is a vertical section.

35 In the drawings in which like letters of reference designate corresponding parts, *a* is an oxy-hydrogen blow-pipe surmounted by a feed reservoir *b*, provided with a suitable support (not shown). This reservoir 40 contains the material to be used, either magnesia, silica, or alumina. The upper end of the main tube of the blow-pipe extends into the reservoir *b* and terminates in a tubular foraminous portion *g* preferably formed of 45 woven wire through which the material contained in the reservoir is adapted to be forced or shaken.

Below the blow-pipe is arranged a vertical screw threaded rod *c*, capable of moving up or down through a distance equal to the length of the filament, which is to be obtained. At the upper end of this screw *c*, is fitted a support *d* of alumina on which the flame of the blow-pipe *a* strikes, to effect the

fusion of the material as the latter reaches it from the reservoir *b*.

The fall of the material is produced by an electric vibrating striker *e*, which produces vibrations which compel the material, previously reduced to a fine powder, to flow through the openings in the tube *g*, down the central tube of the blow-pipe and to fall in a fine thread upon the support *d*. There it fuses, and by causing the said support to move downward in proportion to the amount of product made a filament *f* is obtained the diameter of which is dependent upon the diameter of the opening of the tube, from which the material flows.

To increase the hardness of the filaments, 70 there may be added to the alumina, silica, or magnesia, a certain quantity of oxid of thorium, cerium, or other oxid of this series.

The light produced by the incandescence of the filaments obtained by the process above described may be colored with different colors. This result is obtained by adding to the lime, silica, alumina, or magnesia used to form the filament different metallic oxids. More particularly there may be added 75 oxid of chromium (sesquioxid), which is mixed with the material employed, in suitable proportion, for example 2½ per cent. In this way there is obtained, by the addition of oxid of chromium a color which takes 80 away from the mantles the somewhat greenish appearance which they present, and gives a color very analogous to that of electric lamps.

It is to be understood that, filaments produced in accordance with my invention as hereinbefore set forth, are adapted without alteration to be used as filaments in gas incandescent mantles and as glowers made incandescent by the passage of an electric current. If, in this application, of our process it is desired to increase the conductivity of the filaments for electric lamps, there may be added to the powdered material employed in producing the filaments a certain 95 quantity of powdered vanadium, tantalum, osmium, or other metals of this series.

Having thus described our invention what we claim is,

1. A process of producing filaments from 105 suitable material, which consists in feeding the same in a fine stream in the form of a powder and arresting its movement in a

zone of intense heat to agglomerate the same, whereby a filament of the agglomerated material is produced.

2. A process of producing filaments from suitable material by means of heat, which consists in feeding the material in powdered form to the heat zone in a fine stream, arresting the movement of said stream in said heat zone to produce a filament therefrom and gradually removing the newly formed filament from said point of arrest, whereby the end thereof which is receiving the powdered material will remain in approximately the same position in the heat zone.

15 3. The process of producing filaments from material fusible only at a high temperature which consists in fusing the same in a powdered state in a fine stream, in an

oxy-hydrogen flame and forming the fused material into a filament substantially as described. 20

4. The process of producing filaments which consists in mixing together alumina and oxides of thorium, cerium and chromium, reducing this material to the form of a fine powder, fusing the same in a fine stream and finally forming the fused mass into a filament, substantially as described. 25

In testimony whereof we affix our signatures in presence of two witnesses.

GEORGES MICHAUD.  
EUGÈNE DELASSON.

Witnesses:

EMILE COUCHOND,  
HANSON C. COXE.